

# UNITED STATES PATENT OFFICE.

RAY P. PERRY, OF UPPER MONTCLAIR, NEW JERSEY, ASSIGNOR TO THE BARRETT COMPANY, A CORPORATION OF NEW JERSEY.

## CONSTRUCTION MATERIAL.

1,400,312.

Specification of Letters Patent.

Patented Dec. 13, 1921.

No Drawing.

Application filed September 3, 1920. Serial No. 407,989.

To all whom it may concern:

Be it known that I, RAY P. PERRY, a citizen of the United States, residing at Upper Montclair, in the county of Essex and State 5 of New Jersey, have invented certain new and useful Improvements in Construction Materials, of which the following is a specification.

This invention relates to a construction 10 material and the process of producing the same. It relates more particularly to a construction material containing fibrous material and water proofing material, such for example as pitch, asphalt, and the like. 15 Heretofore it has been well known that sheets of material suitable for roofing, wall boards, etc., can be formed on an ordinary paper making machine. It is also well known that during the paper making process 20 comminuted water proofing material may be introduced into the pulp in the paper making machine and becomes incorporated in the sheet as the sheet is formed. In such sheets the water proofing material may be 25 subsequently fused and caused to spread uniformly by heating or by heating and pressing the same. It has been observed that in the making of such sheets on a paper making machine the fibers arrange themselves in 30 large measure in directions parallel with the longitudinal dimension of the sheet. The fibers may be interlaced or felted together and cross each other to some extent but a large proportion lies in a direction longitudinal 35 of the sheet. In my prior application Ser. No. 398,229, filed July 22, 1920, is described a process by which sheets or layers of mixed fibers and comminuted water proofing material are superposed upon each other 40 and intimately united by heat and pressure.

The present invention is an improvement over the prior art in that the construction material made in accordance with this invention possesses properties not present in 45 the articles heretofore made. One of the main advantages of the present invention is that the article produced has less tendency to be split or fractured and is also less apt to sag after being installed. I take sheets or 50 layers of mixed fibers and water proofing materials that have been formed on a paper making machine and ply the same together so that the fibers in one sheet or layer lie at an angle to the fibers in an adjacent sheet or 55 layer and then intimately unite the sheets by

the application of heat and pressure. It is preferable to assemble the sheets in such a manner that the longitudinal edge of one sheet as it comes from the paper making machine is at right angles to the longitudinal 60 edge of the next sheet, but certain advantages may be obtained by turning the sheets with respect to each other at an angle less than a right angle.

It will be obvious that the pieces or layers 65 cut from the sheet formed on the paper making machine may assume a great variety of shapes such as square, triangular, rectangular, trapezoidal, etc. In every case the pieces or plies will be so assembled that the 70 general direction of the fibers in one piece or ply is at an angle to the general direction of the fibers in the adjacent piece or ply. In case of pieces of certain shapes such as rectangular or otherwise the ends or corners of 75 an overlying sheet will project beyond the edge of the next sheet so that when heat and pressure are applied to produce unification the overhanging portions may not be compressed or densified. As a result of the hot 80 pressing operation the contacting parts become intimately united and form a substantially homogeneous and integral article.

The invention will be more particularly illustrated by the following specific example 85 which is not intended to restrict the invention to the particular materials mentioned. About 20 to 35% of paper making stock such as rag stock, wood fibers, etc., may be mixed with about 80 to 65% by weight of comminuted water proofing material such as pitch of a melting point of 280° F. to 300° F. more or less and formed into a sheet on the paper making machine. A substantial portion of the water may be removed from 90 the sheet, or the sheet may be partially or entirely dried and cut into strips of the desired shape, which strips are assembled so that the general direction of fibers in one strip lie at an angle, preferably a right 95 angle, to the general direction of fibers in the next strip. The group of assembled or laminated strips is then pressed in the presence of sufficient heat to fuse the pitch at such a pressure, say 150 to 300 pounds more or less 100 per square inch, so that the thickness may be reduced to about one-half of the original thickness. The pressure should preferably be applied perpendicular to the sheets so that 105 they will not become torn during the press- 110

ing operation. During this hot pressing operation the waterproofing material flows and covers the surfaces of many of the fibers and cements the same together so that the plane 5 of demarcation between adjacent strips is substantially or entirely obliterated, thus forming an integral homogeneous article. If necessary the strips may be cooled while the pressure is still applied in order for the 10 waterproofing material to "set" so that the article will not expand after the pressure is removed.

It has been found that an article produced in accordance with this invention will with- 15 stand fracture or splitting in a very effective manner and that the tendency for it to sag or bend even when installed on a roof in hot climates or in locations where unusually high atmospheric temperatures are reached is 20 overcome. The degree of hardness and rigidity of the product will depend in large measure upon the proportion of waterproofing material and the melting point of the same. The articles made hereby are found 25 to be substantially impervious to water.

I claim—

1. The process which comprises forming sheets containing fibrous material and waterproofing material so that the fibers lie in one 30 general direction, plying a plurality of such sheets together so that fibers in one sheet are at an angle to those in an adjacent sheet, and heating and pressing the same.

2. The process which comprises forming sheets containing fibrous material and waterproofing material on a paper making machine so that the fibers lie in one general direction, plying a plurality of such sheets together so that fibers in one sheet are at an 40 angle to those in an adjacent sheet, and heating and pressing the same.

3. The process which comprises forming sheets containing fibrous material and waterproofing material so that the fibers lie in one 45 general direction, plying a plurality of such sheets together so that fibers in one sheet cross those in an adjacent sheet, and heating and pressing the same.

4. The process which comprises forming sheets containing fibrous material and waterproofing material so that the fibers lie in one general direction, plying a plurality of such sheets together so that fibers in one sheet are at an angle to those in an adjacent sheet, and uniting 55 said sheets by heat and pressure.

5. The process which comprises forming sheets containing fibrous material and pitch so that the fibers lie in one general direction, plying a plurality of such sheets together so that fibers in one sheet are at an angle to those in an adjacent sheet, and heating and pressing the same.

6. The herein described process which comprises uniting sheets of fibrous material and waterproofing material by heat and pres-

sure, the fibrous material in the individual sheets being somewhat alined and the fibers in one sheet being at an angle to those in an adjacent sheet.

7. The herein described process which 70 comprises uniting sheets of fibrous material and pitch by heat and pressure, the fibrous material in the individual sheets being somewhat alined and the fibers in one sheet being at an angle to those in an adjacent sheet. 75

8. As an article of manufacture, a construction material comprising sheets of mixed fibrous and waterproofing materials which have been united by heat and pressure, the fibers in the sheets being substantially 80 alined and those in one sheet being at an angle to those in an adjacent sheet.

9. As an article of manufacture, a construction material comprising sheets of mixed fibrous and waterproofing materials 85 which have been united by heat and pressure, the fibers in the sheets being substantially alined and those in one sheet being at substantially right angles to those in an adjacent sheet. 90

10. As an article of manufacture, a construction material comprising sheets of mixed fibrous material and pitch which have been united by heat and pressure, the fibers in the sheets being substantially alined and 95 those in one sheet being at an angle to those in an adjacent sheet.

11. As an article of manufacture, a construction material comprising sheets of mixed fibrous and waterproofing materials which 100 have been united by heat and pressure and densified to substantially one-half their original thickness, the fibers in the sheets being substantially alined and those in one sheet being at an angle to those in an adjacent sheet. 105

12. As an article of manufacture, a construction material comprising sheets of mixed fibrous and waterproofing materials in approximately the proportions of 1 to 4 by 110 weight which have been united by heat and pressure, the fibers in the sheets being substantially alined and those in one sheet being at an angle to those in an adjacent sheet.

13. As an article of manufacture, a construction material comprising sheets of mixed fibrous material and pitch of a melting point of approximately 300° F. which have been united by heat and pressure, the fibers in the sheets being substantially alined 120 and those in one sheet being at an angle to those in an adjacent sheet. 115

14. As an article of manufacture, a construction material comprising fibrous and waterproofing materials, the fibers being largely alined in layers with the fibers in one layer generally at an angle to those in another layer. 125

In testimony whereof I affix my signature.  
RAY P. PERRY.